

Dec. 7, 1926.

1,610,019

W. H. LOWE

PAVEMENT

Filed Oct. 26, 1925

22 21 FIG. 5.

FIG. 1.



4 3 6 7



FIG. 2.

FIG. 3.



14 12 13 16 7 9 8 7



FIG. 4.



INVENTOR  
William H. Lowe  
By Charles S. Evans  
Attorney

## UNITED STATES PATENT OFFICE.

WILLIAM H. LOWE, OF SAN FRANCISCO, CALIFORNIA, ASSIGNOR TO THE PARAFFINE COMPANIES, INC., OF SAN FRANCISCO, CALIFORNIA, A CORPORATION OF DELAWARE.

## PAVEMENT.

Application filed October 26, 1925. Serial No. 64,805.

My invention relates to floors and pavements, and one of the objects of the invention is the provision of a structure of special adaptability as a flooring for industrial uses, or as a paving of general application and which is characterized by economy and great durability.

Another object of the invention is the provision of a flooring or paving which is vermin- and decay-proof and also water-, acid-, and alkali-proof.

Another object of the invention is the provision of a flooring or paving having a certain measure of resilience.

Another object is the provision of a flooring or paving which deadens and absorbs vibration and prevents noise.

Another object of my invention is the provision of a flooring or paving which lends itself readily to permanent markings to indicate safety zones, parking places and other areas, or to give information or directions.

My invention possesses other objects and features of advantage some of which with the foregoing will be set forth in the following description of the preferred embodiment of means for practicing the invention which is illustrated in the drawings accompanying and forming part of the specification. It is to be understood that I do not limit myself to the showing made by the said description and drawings as I may adopt variations of my preferred form within the scope of my invention as set forth in the claims.

Referring to the drawings:

Figure 1 is a vertical section thru a portion of my flooring or paving structure in its preferred and simplest form.

Figure 2 is a plan view of a section of my pavement as used to indicate a safety zone.

Figure 3 is a vertical section thru a portion of floor or pavement embodying a variant form of my invention.

Figure 4 is a vertical sectional view thru the pavement shown in Figure 2. The plane on which the section is taken is indicated by the line 4-4 of Figure 2.

Figure 5 is a vertical sectional view similar to Figure 4 but showing another embodiment of my invention.

In terms of broad inclusion my invention comprises a flooring or pavement which is structurally a single unit after it is laid, and which comprises one or more layers overlying a substructure or base. The layers consist of fibrous sheets which have been saturated with a semi-solid material to render the sheet slightly and slowly yieldable under impact. A similar material is used to cement together the layers or sheets, if there be more than one, and the sheet or sheets to the underlying substructure or base. Where it is desired to mark the pavement to indicate safety zones or for other purposes, strips or pieces of different color than that of the body of the pavement are interposed therein, or laid thereon, and these strips or pieces may be the letters of words or used as lines.

In greater detail the flooring of my invention comprises a base structure 2 of concrete, wood or other suitable material commonly used for the purpose. Overlying the substructure or base is a layer 3 of fibrous material, such as a rag felt sheet which I have found convenient to make of, say, 80% rag, 10% burlap, and 10% of other fiber such as redwood bark. This sheet is saturated with a bituminous compound, semi-solid at ordinary temperatures, and is also provided on the upper or on both sides with a coating 4 of bitumen, solid at ordinary temperatures, and having a melting point of about 180° F. This coating is on the upper or wearing surface of the flooring, and coalesces more or less with the saturating compound.

The sheet 3 is united with the sub-structure 2 by a layer 6 of bituminous cement, preferably a relatively hard steam-blown asphalt dissolved in carbon bisulfide, benzole, or other suitable solvent. This layer penetrates into the fibers or the grain of the underlying base structure and also coalesces and unites with the saturant or coating of the sheet, so that the sub-structure and overlying sheet are substantially unitary in form. This results in a structure having a rigid non-resilient base faced with a wearing layer of slightly and slowly yieldable material, having a measure of resilience but yet not springy, capable of slow flow under pressure in a minor degree and within nar-

row limits, and yet firm under the impact of the feet or wheels.

Because of the coating and underlying saturant with which it integrally unites, my flooring or pavement possesses a very peculiar and valuable property, namely that of "healing" over minor injuries in the surface. As a flooring, it is particularly designed for industrial uses and finds its chief application in locations where it is subjected to most destructive wear, such for example as canneries, restaurants, laundries, street-car platforms and floors, ice and cold storage plants, refrigerator cars, laboratories, granaries, malt houses and grain elevators, offices and schoolrooms. It is also applicable to corridors and sidewalks, and to mark quiet zones and tennis courts. As a pavement it is particularly valuable on bridges and their approaches, streets adjacent hospitals and churches.

In such uses as these, it is subjected to the wearing action of heavy shoes, loaded trucks, falling objects, vehicular traffic and other destructive influences; many of which inflict actual mechanical injury to the surface. Possessing the peculiar property just mentioned, ordinary cuts and injuries of relatively minor character quickly fill up and level over, due to the slow flowing of the saturating and coating materials under conditions of use, so that substantially an even and smooth surface is restored by wear.

The fibrous character of the saturated sheet and the property of slowly giving or yielding under impact makes my flooring or paving a resilient one without any perceptible springiness and growing out of the same qualities is another desirable feature, that of quietness. My flooring or paving absorbs vibration and is without resonance, and hence even the running of trucks over it is unaccompanied by any of the noises associated with wood or concrete floors.

My flooring or paving is characterized by extreme durability, in actual tests on a car loading platform, sections of it having out-worn steel plate. One of the reasons for its extreme durability is believed to lie in the fact that the saturation of the fibrous sheet in a semi-solid material prevents what may be termed "internal wear", that is, the mutually destructive action of fibers crushed together, while at the same time permitting a sufficient "give", or yielding, under shock, to preserve a certain measure of resilience. Further, the cementing of the sheet to a rigid base so that a unitary structure results, prevents any lateral slipping of the fibrous sheet and narrowly localizes shocks and stresses.

Because of the chemical characteristics of the saturant and coating materials, my flooring or paving is vermin-proof, decay-proof, and water-, acid-, and alkali-proof.

I have found that a very durable floor or pavement and one which is relatively cheap to lay, may be made with a fibrous sheet comprising a heavy prepared roofing, and this flooring is black to dark grey in color. 70 Instead of coating my fibrous sheet as above noted, I may use a coating composed of 55% light colored stearin pitch, 10% of gilsonite, 5% petroleum or wool grease and 30% finely divided red iron oxide. This gives 75 a red coating substantially similar to the one first explained except that it has a slightly lower melting point, altho solid at all ordinary temperatures.

The structure above described is the preferred and simplest embodiment of my invention, but in Figure 3, I have shown another embodiment, in which the maximum of all of the desirable qualities is secured. The floor or pavement as illustrated in this 80 figure comprises the base or substructure 2, over which a thin layer 7 of dampcourse is laid, and united to the base by a layer 8 of bituminous cement. The cracks 9 between the layers 7 are also filled with the bituminous cement, and over the layers of dampcourse are cemented, by the layer 12 of bituminous cement, the relatively heavy fibrous sheet 13 similar to the sheet 3 first explained. The dampcourse comprises preferably a sheet similar to the sheet 13 but made of thinner material. The cracks 14 between these sheets are also filled with the bituminous cement compound, so that both the overlying sheet 13, the intervening sheet 90 7 and the substructure 2 are integrally united into a unitary structure. The overlying sheets 13 are provided with a coating 16 similar to the coating 4 described in connection with the structure shown in Figure 1. 105

In laying this flooring or paving it is desirable of course to break joints between the layers 7 and 13 as shown in the drawing.

The flooring or paving shown in Figure 3 is a trifle more expensive to lay than the one first explained, but this is more than compensated by the increase in desirable qualities, of noiselessness, extreme durability and water-proofness.

If desired, creosote may be incorporated 110 in the saturant and zinc sulfate in the felt, either or both, to inhibit the growth of fungus or destructive micro-organisms in general. In certain uses of my flooring these qualities would add to its value and usefulness, and because of the more exposed location usual in a pavement, I prefer to treat in this manner the materials going into a pavement or sidewalk.

In Figure 2, I have shown a plan view 125 of a pavement embodying my invention and marked for a safety zone. The body of the pavement 17 is laid as already explained, for example, in connection with Figure 1. A strip 18 is then cut from similar material 130

of a different and preferably lighter color, and is inlaid into the body 17 of the pavement as shown in Figure 4, the abutting edges being carefully cemented together by a layer or body 19 of bituminous or other suitable cement.

In some cases I prefer to overlay the body of my pavement with an added piece as shown in Figure 5, comprising a piece of fibrous material similar to that already referred to; or comprising a fabric strip having a dense rag felt base 21, saturated with a bituminous compound and having a wearing coating 22 over the exposed surface.

15 This coating is of the enamel type of paint in which a light pigment predominates, and is baked on. It provides a surface which is semi-flexible and extremely tough, and highly resistant to wear.

20 A satisfactory strip for marking a pavement in this manner has been made from a good grade of so-called "printed floor covering". The strip is secured in place preferably by a bituminous cement.

25 In the following claims I shall use the term "pavement" to designate my new structure

whether it is applied to floor, sidewalk, or street use.

I claim:

1. A pavement comprising a supporting substructure, and overlying fibrous sheet adhesively united to the substructure, the fibrous sheet being saturated with a semi-solid material to render the sheet slightly and slowly yieldable under impact and being coated on its exposed surface with a bituminous compound solid at normal temperatures but capable of coalescing after scarring. 30

2. A pavement comprising a supporting base, an overlying fibrous sheet saturated with a semi-solid bituminous material to render it slightly and slowly yieldable under impact, and coated on its exposed surface with a bituminous compound solid at normal 35 temperatures but capable of coalescing after scarring, and an intervening cementing layer of bituminous compound to bind the whole into a unitary structure. 45

In testimony whereof, I have hereunto set my hand. 50

WILLIAM H. LOWE.